# EUROPEAN PATENT SPECIFICATION

(11) **EP 0 376 311 B1**
(45) Date of publication and mention of the grant of the patent: **05.04.1995**
(21) Application number: 89124079.8
(22) Date of filing: 28.12.1989
(51) Int. Cl.: G03G 5/06

(54) **Photosensitive member for electrophotography**
Lichtempfindliches Element für Elektrophotographie
Elément photosensible pour électrophotographie

(30) Priority: 29.12.1988 JP 330987/88; 29.12.1988 JP 330995/88
(43) Date of publication of application: 04.07.1990
(73) Proprietor: CANON KABUSHIKI KAISHA, Tokyo (JP)
(72) Inventor: Kikuchi, Toshihiro, Yokohama-shi Kanagawa-ken (JP); Kanemaru, Tetsuro, Tokyo (JP); Senoo, Akihiro, Yokohama-shi Kanagawa-ken (JP); Yashiro, Ryoji, Higashiyatsushiro-gun, Yamanashi-ken (JP)
(74) Representative: Bühling, Gerhard, Dipl.-Chem.

(56) References cited:
- EP-A- 0 161 934
- US-A- 4 869 988
- PATENT ABSTRACTS OF JAPAN vol. 13, no. 89 (P-836)(3437) 02 March 89,& JP-A-63 271355
- PATENT ABSTRACTS OF JAPAN vol. 12, no. 231 (P-723)(3078) 30 June 1988 & JP-A-63 23162

## Description

### FIELD OF THE INVENTION AND RELATED ART

The present invention relates to a photosensitive member for electrophotography, particularly to a photosensitive member for electrophotography comprising a low-molecular weight organic photoconductor capable of providing improved electrophotographic characteristics.

Hitherto, there have been proposed a large number of organic photoconductive polymers to be used for electrophotographic photosensitive members, such as polyvinyl carbazole. These conventional organic polymers are superior to inorganic photoconductive materials in lightness (in weight), film-forming property, etc., but are inferior to the latter in sensitivity, durability, stability to environmental change, mechanical strength, etc.

On the other hand, there have been proposed several low-molecular weight organic photoconductive materials such as hydrazone compound (U.S. Patent 4,150,987), triaryl pyrazoline compound (U.S. Patent 3,837,851), and 9-styryl anthracene (Japanese Laid-Open Patent Application (JP-A, KOKAI) Nos. 94828/1976 and 94829/1976).

In a case where the conventional low-molecular weight organic photoconductors represented by those as described above are used, the above-mentioned defect in film-forming property, which has conventionally posed a problem in the field of the organic photoconductive polymer, may be obviated by appropriately selecting a binder to be used in combination therewith. However, these conventional organic photoconductors cannot provide a sufficient sensitivity.

In such a viewpoint, there has recently been proposed a laminate-type structure wherein the photosensitive layer is function-separated into a charge generation layer and a charge transport layer. The electrophotographic photosensitive member comprising such a photosensitive layer may be improved in sensitivity to visible light, charge retentivity, surface strength, etc.

As the charge-transporting substance constituting the above-mentioned charge transport layer, a large number of organic compounds have heretofore been proposed. Examples thereof include: pyrazoline compounds (Japanese Laid-Open Patent Application No. 72231/1977), hydrazone compounds (U.S. Patent 842,431 and Japanese Laid-Open Patent Application No. 52063/1980), triphenylamine compounds (Japanese Laid-Open Patent Application Nos. 195254/1982 and 58445/1979), stilbene compounds (Japanese Laid-Open Patent Application Nos. 151955/1979 and 198043/1983), carbazole compounds (Japanese Laid-Open Patent Application Nos. 150128/1979 and 58451/1988), benzothiophene compounds (Japanese Laid-Open Patent Application No. 110835/1979), etc.

The EP-A-0 161 934 discloses an electrophotographic photosensitive member, the charge transporting layer of which contains a charge transporting aromatic amine compound represented by the general formula:
wherein R₁ and R₂ are an aromatic group selected from the group consisting of a substituted or unsubstituted phenyl group, naphthyl group and polyphenyl group and R₃ is selected from the group consisting of a substituted or unsubstituted aryl group, alkyl group having from 1 to 18 carbon atoms and cycloaliphatic compounds having from 3 to 18 carbon atoms.

However, in the electrophotographic photosensitive member using the conventional low-molecular weight organic compound as the charge-transporting substance, the sensitivity and other electrophotographic characteristics are not necessarily sufficient, and the light part potential and dark part potential are liable to show a considerable change, when charging and exposure operations are conducted repetitively.

Accordingly, with respect to such an electrophotographic photosensitive member, there is still room for improvement.

### SUMMARY OF THE INVENTION

An object of the present invention is to provide an electrophotographic photosensitive member which has solved the above-mentioned various problems encountered in the conventional photosensitive member.

Another object of the present invention is to provide an electrophotographic photosensitive member using a novel organic photoconductor which may easily be produced, is relatively inexpensive and is excellent in durability.

According to the present invention, there is provided a photosensitive member for electrophotography, comprising an electroconductive substrate and a photosensitive layer disposed thereon, wherein the photosensitive layer comprises a triarylamine compound represented by the following general formula (I) or (II):
wherein Ar₁ and Ar₂ respectively denote a biphenyl group capable of having a substituent; Ar₃ denotes a phenyl group capable of having a substituent or an aromatic heterocyclic group capable of having a substituent; Ar₄ and Ar₅ respectively denote a benzene ring capable of having a substituent or aromatic fused-ring hydrocarbon group capable of having a substituent; R₁ and R₂ respectively denote a hydrogen atom, alkyl, alkoxyl or halogen atom; and at least one of Ar₄ and Ar₅ is an aromatic fused-ring hydrocarbon group.

In claim 1 for the contracting stated DE, Ar₃ of formula (I) is specified to denote only an aromatic hetero cyclic group capable of having a substituent in view of the earlier national right DE-A-38 35 791.

These and other objects, features and advantages of the present invention will become more apparent upon a consideration of the following description of the preferred embodiments of the present invention taken in conjunction with the accompanying drawings.

### BRIEF DESCRIPTION OF THE DRAWINGS

Figures 1 and 2 show infrared absorption spectra of Compound Example Nos. 2 and 26, respectively, according to the KBr tablet method.

### DETAILED DESCRIPTION OF THE INVENTION

In the above general formula (I), Ar₁ and Ar₂ respectively denote a biphenyl group capable of having a substituent. Specific examples of such a substituent may include alkyl groups such as methyl, ethyl and propyl; alkoxy groups such as methoxy, ethoxy and propoxy; halogen atoms such as fluorine, chlorine and bromine; etc. Ar₁ may be the as or different from Ar₂.

Ar₃ denotes a phenyl group capable of having a substituent, or an aromatic heterocyclic group such as pyridyl, quinolyl, thienyl or furyl capable of having a substituent. Specific examples of such a substituent may include: alkyl groups such as methyl, ethyl and propyl; alkoxy groups such as methoxy, ethoxy and propoxy; aryloxy groups such as phenoxy and naphthoxy; aromatic groups such as phenyl and naphthyl; halogen atoms such as fluorine, chlorine and bromine; etc.

In the above general formula (II), Ar₄ and Ar₅ respectively denote a benzene ring or aromatic condensed-ring (or fused-ring) hydrocarbon group capable of having a substituent. At least one of Ar₄ and Ar₅ an aromatic condensed ring hydrocarbon group. Specific examples of such an aromatic condensed ring hydrocarbon may include naphthalene, anthracene, phenanthrene, chrysene and naphthacene. Specific examples of such a substituent which Ar₄ and Ar₅ may have include: alkyl groups such as methyl, ethyl and propyl; alkoxy groups such as methoxy, ethoxy and propoxy; halogen atoms such as fluorine, chlorine and bromine; etc. Ar₄ may be the as or different from Ar₅.

R₁ and R₂ respectively denote a hydrogen atom; an alkyl group such as methyl, ethyl and propyl; an alkoxy group such as methoxy, ethoxy and propoxy; a halogen atom such as fluorine, chlorine and bromine; etc. R₁ may be the as or different from R₂.

Representative examples of the compound represented by the above-mentioned formula (I) are described hereinbelow.

### <Compound Examples>

Representative examples of the compound represented by the above-mentioned formula (II) are described hereinbelow.

### <Compound Examples>

The above-mentioned Compound Examples may be synthesized in the following manner.

### <Synthesis of Compound Example No. 2>

23.5 g (83.9 mmol) of 4-iodobiphenyl, 3.0 g (28.0 mmol) of p-toluidine, 11.6 g (83.9 mmol) of anhydrous potassium carbonate, and 15 g of copper powder were added to 50 ml of nitrobenzene, and refluxed for 12 hours under heating and stirring. After the reaction mixture was cooled, the reaction mixture was subjected to filtration by suction, and the nitrobenzene was removed from the resultant filtrate under reduced pressure. Ethanol was added to the residue to precipitate crude crystals.

The crude crystals were subjected to separation to be purified by using a silica gel column, whereby 7.80 g (yield = 66.7 %) of the intended Compound Example (2) showing a melting point of 187.0 - 188.0 °C was obtained.

Figure 1 shows an infrared absorption spectrum chart obtained by measuring the thus obtained compound by a KBr tablet (or pellet) method.

### <Synthesis of Compound Example No. 26>

5.75 g (20.5 mmol) of 4-iodobiphenyl, 3.0 g (13.7 mmol) of N-phenyl-α-naphthylamine, 2.83 g (20.5 mmol) of anhydrous potassium carbonate, and 1.5 g of copper powder were added to 30 ml of nitrobenzene, and refluxed for 10 hours under heating and stirring. After the reaction mixture was cooled, the reaction mixture was subjected to filtration by suction, and then the nitrobenzene was removed from the resultant filtrate under reduced pressure. The residue was subjected to separation to be purified by using a silica gel column, whereby 3.3 g (yield = 65 %) of the intended Compound Example (26) showing a melting point of 176.5 - 177.5 °C was obtained.

Figure 2 shows an infrared absorption spectrum chart obtained by measuring the thus obtained compound by a KBr tablet (or pellet) method.

As described above, the compound according to the present invention may easily be synthesized inexpensively. The other compounds according to the present invention may be synthesized in a similar manner as described in the above-mentioned Synthesis Examples.

In a preferred embodiment of the present invention, the photosensitive layer is function-separated into a charge generation layer and a charge transport layer, and the charge transport layer comprises the compound represented by the above-mentioned general formula (I) or (II) as a charge-transporting substance.

The charge transport layer according to the present invention may preferably be formed by dissolving the above-mentioned compound of the formula (I) or (II) in an appropriate solvent together with a binder, applying the resultant coating liquid such as solution onto a predetermined surface, and drying the resultant coating.

Examples of the binder to be used for forming the charge transport layer may include; polyarylate resins, polysulfone resins, polyamide resins, acrylic resins, acrylonitrile resins, methacrylic resins, vinyl chloride resins, vinyl acetate resins, phenol resins, epoxy resins, polyester resins, alkyd resins, polycarbonate, polyurethane, or copolymer resins containing two or more of the recurring units of these resins, such as styrene-butadiene copolymers, styrene-acrylonitrile copolymers, styrene-maleic acid copolymers, etc. Also, other than such insulating polymers, organic photoconductive polymers such as polyvinylcarbazole, polyvinylanthracene and polyvinylpyrene may be used.

In the charge transport layer, the charge-transporting substance may preferably be used in an amount of 10 - 500 wt. parts, more preferably 50 - 200 wt. parts, per 100 wt. parts of the binder.

The charge transport layer is electrically connected to the charge generation layer as described hereinafter, and has a function of receiving charge carriers injected from the charge generation layer in the presence of an electric field and of transporting these charge carriers to the surface of the charge transport layer. In such an embodiment, the charge transport layer may be disposed on the charge generation layer, or may be disposed under the charge generation layer. The charge transport layer may preferably be disposed on the charge generation layer. It is not preferred that the charge transport layer has too large a thickness, since there is a certain limit to the thickness thereof suitable for the transport of the charge carriers. In general, the charge transport layer may preferably have a thickness of 5 - 40 microns, more preferably 10 - 30 microns.

The organic solvent to be used in the above-mentioned formation of the charge transport layer may vary depending on the kind of the binder used therefor, and may preferably be selected from those which do not substantially dissolve the charge generation layer or a primer (or undercoat layer) as described hereinafter.

Specific examples of such an organic solvent may include: alcohols such as methanol, ethanol, and isopropanol; ketones such as acetone, methyl ethyl ketone, and cyclohexanone; amides such as N,N-dimethylformamide and N,N-dimethylacetamide; sulfoxides such as dimethyl sulfoxide; ethers such as tetrahydrofuran, dioxane, and ethylene glycol monomethyl ether; esters such as methyl acetate and ethyl acetate; aliphatic halogenated hydrocarbons such as chloroform, methylene chloride, dichloroethylene, carbon tetrachloride, and trichloroethylene; aromatic compounds such as benzene, toluene, xylene, monochlorobenzene, and dichlorobenzene; etc.

The coating may be effected by various coating methods such as dip coating, spray coating, wire bar coating, and blade coating. The drying should preferably be conducted in the sequence of drying at room temperature to a "tack-free" state and then heat drying. In general, the heat drying may preferably be conducted for a time in the range of 5 minutes to 2 hours at a temperature of 30 °C to 200 °C under quiescent condition or under blowing.

The charge transport layer according to the present invention can further contain an additive selected from various species thereof. Examples of such an additive may include: plasticizers such as diphenyl, m-terphenyl and dibutyl phthalates; surface-lubricating agents such as silicone oil, graft-type silicone polymers, and various fluorocarbons; potential stabilizing agents such as dicyanovinyl compounds and carbazole derivatives; anti-oxidizing agents such as β-carotene, Ni complexes, and 1,4-diazabicyclo[2,2,2]-octane; etc.

The charge generation layer may comprise a charge-generating substance. Specific examples of the charge-generating substance may include: inorganic charge-generating substances such as selenium, selenium-tellurium, and amorphous silicon; and organic charge-generating substances including: cationic dyes such as pyrylium dye, thiapyrylium dye, azulenium dye, thiacyanine dye, and quinocyanine dye; polycyclic quinone pigments such as squarium salt dye, phthalocyanine pigment, anthanthrone pigment, dibenzpyrene-quinone pigment, and pyranthrone pigment; indigo pigment; quinacridone pigment; azo pigment; etc. These charge-generating substances may be used singly or as a combination of two or more species. The charge generation layer may be formed by using such a charge-generating substance in the form of a vapor deposition layer or coating layer.

Among the above-mentioned charge-generating substances, the azo pigment particularly includes various types. Representative structures of the azo pigment preferably used in the present invention are described hereinbelow. When the azo pigment is represented by a general formula including the following central skeleton A:

A(̵N=N-Cp)ₙ

wherein Cp denotes a coupler portion (or coupler moiety) and n is 2 or 3, specific examples of the central skeleton A include those comprising the following structures:

Specific examples of the coupler portion Cp include those having the following structures:

The above-mentioned central skeleton A and coupler Cp may appropriately be combined to form a pigment as a charge-generating substance.

The charge generation layer may be formed by vapor-depositing such a charge-generating substance by means of a vacuum vapor deposition device, or by applying a dispersion containing such a charge-generating substance dispersed therein, together with an appropriate binder as desired.

The binder to be used for forming the charge generation layer may be selected from a wide variety of insulating resins or alternatively from organic photoconductive polymers such as poly-N-vinylcarbazole, polyvinylanthracene, and polyvinylpyrene. There may preferably be used the insulating resin such as polyvinyl butyral, polyarylates (e.g., polycondensation product between bisphenol A and phthalic acid), polycarbonate, polyester, phenoxy resin, acrylic resin, polyacrylamide resin, polyamide, polyvinyl pyridine, cellulose resin, urethane resin, epoxy resin, casein, polyvinyl alcohol, and polyvinyl pyrrolidone.

The resin may preferably be contained in the charge generation layer in an amount of 5 - 80 wt. %, more preferably 10 - 40 wt. %.

Specific examples of the organic solvent usable in the coating of the charge generation layer may include: alcohols such as methanol, ethanol, and isopropanol; ketones such as acetone, methyl ethyl ketone, and cyclohexanone; amides such as N,N-dimethylformamide and N,N-dimethylacetamide; sulfoxides such as dimethyl sulfoxide; ethers such as tetrahydrofuran, dioxane, and ethylene glycol monomethyl ether; esters such as methyl acetate and ethyl acetate; aliphatic halogenated hydrocarbons such as chloroform, methylene chloride, dichloroethylene, carbon tetrachloride, and trichloroethylene; aromatic compounds such as benzene, toluene, xylene, monochlorobenzene, and dichlorobenzene; etc.

The charge generation layer may preferably contain the above-mentioned charge-generating substance in an amount as large as possible, so that it may provide a sufficient absorbance. Further, the charge generation layer may preferably be a thin layer having a thickness of 5 microns or below, more preferably 0.01 - 1 micron so that it may inject charge carriers generated therein into the charge transport layer within the lifetime of the charge carriers. This may be attributable to facts such that most of the incident light quantity may preferably be absorbed into the charge generation layer to generate a large number of charge carriers, and that the thus generated charge carriers may preferably be injected into the charge transport layer without deactivation due to recombination or trapping thereof.

The above-mentioned photosensitive layer having a laminate structure comprising a charge generation layer and a charge transport layer may be disposed on an electroconductive substrate.

The electroconductive substrate may be a substrate which per se has an electroconductivity such as those of aluminum, aluminum alloy, copper, zinc, and stainless steel; alternatively, the above-mentioned metal substrate or a substrate of a plastic coated with, e.g., a vacuum vapor-deposited layer of aluminum, aluminum alloy, indium oxide, tin oxide or indium oxide-tin oxide alloy, or a mixture of an electroconductive powder (such as aluminum powder, titanium oxide, tin oxide, zinc oxide, carbon black and silver particles) and an appropriate binder; a substrate of paper or plastic impregnated with electroconductive particles, or a plastic substrate coated with an electroconductive polymer layer. The electroconductive substrate may be in any form such as sheet, drum, etc.

Between the electroconductive substrate and the photosensitive layer, there can be formed a primer or undercoat layer having a barrier function and an adhesive function. The primer layer may comprise, e.g., casein, polyvinyl alcohol, nitrocellulose, ethylene-acrylic acid copolymer, polyamide (e.g., nylon 6, nylon 66, nylon 610, copolymer nylon, alkoxymethylated nylon, etc.), polyurethane, gelatin, or aluminum oxide. The thickness of the primer layer should preferably be 0.1 - 5 microns, particularly 0.5 to 3 microns.

In the electrophotographic photosensitive member according to the present invention, a protective layer can further be disposed on the photosensitive layer. Such a protective layer may comprise a resin, or a resin and an electroconductive material dispersed therein.

In another embodiment of the present invention, a pigment or dye having a photoconductivity may be used as a sensitizer. Examples of such a dye or pigment include: the above-mentioned disazo pigment, pyrylium dye, thiapyrylium dye, selenapyrylium dye, benzopyrylium dye, benzothiapyrylium dye, naphthopyrylium dye, and naphthothiapyrylium dye, as described in U.S. Patent 3,554,745; 3,567,438; and 3,586,500.

In a still another embodiment of the present invention, an eutectic (crystal) complex comprising a pyrylium dye (as disclosed in U.S. Patent 3,684,502) and an electrically insulating polymer comprising an alkylidene-diarylene portion may be used as a sensitizer. Such an eutectic complex may be formed by dissolving 4-[4-bis(2-chloroethyl)aminophenyl]-2,6-diphenylthiapyrylium perchlorate and poly(4,4′-isopropylidene diphenylene carbonate) in a halogenated hydrocarbon-type solvent (e.g., dichloromethane, chloroform, carbon tetrachloride, 1,1-dichloroethane, 1,2-dichloroethane, 1,1,2-trichloroethane, chlorobenzene, bromobenzene, 1,2-dichlorobenzene, etc.), and then adding a non-polar solvent (e.g., hexane, octane, decane, 2,2,4-trimethylbenzene, ligroin, etc.) to the resultant mixture so as to produce a particulate eutectic complex. In such an embodiment, the electrophotographic photosensitive member may include a binder such as styrene-butadiene copolymer, silicone resin, vinyl resin, vinylidene chloride-acrylonitrile copolymer, styrene-acrylonitrile copolymer, vinyl acetate-vinyl chloride copolymer, polyvinyl butyral, polymethyl methacrylate, poly-N-butyl methacrylate, polyester, cellulose ester, etc.

The electrophotographic photosensitive member according to the present invention may be used not only for ordinary copying machines but also in the fields related to electrophotography such as laser printers, CRT printers and electrophotographic plate-making.

The present invention will be described in more detail with reference to Examples.

### Example 1

5 g of a disazo pigment represented by the following formula:
and a solution obtained by dissolving 2 g of a butyral resin (butyral degree: 63 mol. %) in 100 ml of cyclohexanone were dispersed for 24 hours by means of a sand mill to prepare a coating liquid. The thus prepared coating liquid was applied onto an aluminum sheet by means of a wire bar to form a charge generation layer having a thickness (after drying) of 0.2 micron.

Then, 10 g of the above-mentioned Compound Example No. 6 as a charge-transporting substance, and 10 g of a polycarbonate resin (weight-average molecular weight = 20,000) were dissolved in 70 g of monochlorobenzene to prepare a coating liquid. The coating liquid was applied onto the above-mentioned charge generation layer by means of a wire bar to form a charge transport layer having a thickness (after drying) of 20 microns, whereby an electrophotographic photosensitive member having a laminate structure was prepared.

The thus prepared photosensitive member was charged by using corona (-5 KV) according to a static method by means of an electrostatic copying paper tester (Model: SP-428, mfd. by Kawaguchi Denki K.K.) and retained in a dark place for 1 sec. Thereafter, the photosensitive member was exposed to light at an illuminance of 20 lux, to evaluate the charging characteristic. In order to evaluate the charging characteristic, the surface potential (V₀), the potential (V₁) obtained after a dark decay of 1 sec, and the exposure quantity (E_{1/2}) required for decreasing the potential V₁ to 1/2 thereof were measured.

Further, in order to measure the variations in light part potential and dark part potential in repetitive use, the photosensitive member prepared in this instance was bonded to the cylinder for a photosensitive drum to be used for a plain paper copying (PPC) machine (NP-3525, mfd. by Canon K.K.) and subjected to a copying test of 5000 sheets. Thus, the light part potential (V_{L}) and dark part potential (V_{D}) were measured in the initial stage and after the copying of 5000 sheets to evaluate variations therein. The initial V_{D} and V_{L} were set to -700 V and -200 V, respectively.

The results are shown in the following Table 1.

### Example 2

An electrophotographic photosensitive member was prepared in the same manner as in Example 1 except that Compound Example (29) was used as the charge-transporting substance instead of the Compound Example (6) used in Example 1.

The electrophotographic characteristic of the thus obtained photosensitive member were measured in the same manner as in Example 1.

The results are shown in the following Table 2.

### Examples 3 - 11

Nine species of photosensitive members were prepared in the same manner as in Example 1 except that Compound Examples (1), (2), (5), (8), (10), (12), (15), (20) and (23) were respectively used as the charge-transporting substance instead of the Compound Example (6) used in Example 1, and that a pigment having the following formula was used as the charge-generating substance.

The electrophotographic characteristics of the thus obtained photosensitive members were measured in the same manner as in Example 1.

The results are shown in the following Table 3.

### Examples 12 - 17

Six species of photosensitive members were prepared in the same manner as in Example 1 except that Compound Examples (26), (28), (33), (39), (43) and (44) were respectively used as the charge-transporting substance instead of the Compound Example (29) used in Example 2, and that the pigment used in Examples 3 - 11 was used as the charge-generating substance.

The electrophotographic characteristic of the thus obtained photosensitive members were measured in the same manner as in Example 1.

The results are shown in the following Table 4.

### Comparative Examples 1 - 5

For the purpose of comparison, five species of photosensitive members were prepared in the same manner as in Example 1 except that the following Comparative Compound Examples 1 - 5 were respectively used as the charge-transporting substance.

The electrophotographic characteristics of the thus obtained photosensitive members were measured in the same manner as in Example 1.

The results are shown in the following Table 5.

### <Comparative Compound Examples>

As apparent from the results as described above, the compound according to the present invention provided photosensitive member providing a better sensitivity and better potential stability in successive copying, as compared with those of Comparative Examples.

### Examples 18 and 19

A coating liquid obtained by dissolving 5 g of a methoxymethylated nylon resin (number-average molecular weight = 32,000) and 10 g of an alcohol-soluble copolymer nylon resin (number-average molecular weight = 29,000) in 95 g of methanol was applied onto an aluminum substrate by means of a wire bar to form a primer layer having a thickness of 1 micron (after drying).

Then, 10 g of a charge-generating substance represented by the following formula:
a butyral resin (butyral degree: 63 mol. %) and 200 g of dioxane were dispersed for 48 hours by means of a ball mill disperser to prepare a dispersion. The thus prepared dispersion was applied onto the above-mentioned primer layer by a blade coating method to form a charge generation layer having a thickness (after drying) of 0.15 micron.

Then, 10 g of the above-mentioned Compound Example No. 3 and 10 g of a polymethyl methacrylate resin (weight-average molecular weight = 50,000) were dissolved in 70 g of monochlorobenzene to prepare a coating liquid. The coating liquid was applied onto the above-mentioned charge generation layer by a blade coating method to form a charge transport layer having a thickness (after drying) of 19 microns, whereby an electrophotographic photosensitive member was prepared (Example 18).

The thus prepared photosensitive member was charged by using corona discharge (-5 KV) so as to have an initial potential of V₀, left standing in a dark place for 1 sec, and thereafter the surface potential thereof (V₁) was measured. In order to evaluate the sensitivity, the exposure quantity (E_{1/2}, »J/cm²) required for decreasing the potential V₁ after the dark decay to 1/2 thereof was measured. The light source used herein was laser light (output: 5 mW, emission wavelength: 780 nm) emitted from a ternary semiconductor comprising gallium/aluminum/arsenic.

The results were as follows:
V₀: -701 V
V₁: -693 V
E_{1/2}: 0.51 »J/cm²

Separately, the above-mentioned procedure was repeated except that Compound Example No. 41 was used as the charge-transporting substance contained in the charge transport layer, thereby to prepare another electrophotographic photosensitive member. The thus prepared photosensitive member was evaluated in the same manner as described above (Example 19).

The results were as follows:
V₀: -700 V
V₁: -694 V
E_{1/2}: 0.54 »J/cm²

Each of the above-mentioned photosensitive member was assembled in a laser beam printer (trade name: LBP-CX, mfd. by Canon K.K.) as an electrophotographic printer equipped with the above-mentioned semiconductor laser using a reversal development system, and subjected to actual image formation.

The image formation conditions used herein were as follows:
surface potential after primary charging: -700 V
surface potential after image exposure: -150 V
(exposure quantity: 2.0 »J/cm²)
transfer potential: +700 V
polarity of developer: negative
process speed: 50 mm/sec
developing condition (developing bias): -450 V
image exposure scanning system: image scan exposure prior to the primary charging: 50 lux.sec
(whole surface exposure using red light)

The image formation was effected by line-scanning the laser beam corresponding to character and image signals. As a result, good prints were obtained with respect to the characters and images, when each of the above-mentioned two photosensitive members was used.

Further, when successive image formation of 3,000 sheets was conducted, good prints were stably obtained from the initial stage to 3,000 sheets, in a case where each of the above-mentioned two photosensitive members was used.

### Examples 20 and 21, Comparative Examples 6 and 7

10 g of oxytitanium phthalocyanine and a solution obtained by dissolving 5 g of a phenoxy resin in 485 g of dioxane were dispersed for 2 hours by means of a ball mill. The thus prepared dispersion was applied onto an aluminum sheet by means of a wire bar and then dried at 80 °C for 2 hours to form a charge generation layer having a thickness of 0.5 micron.

Then, 10 g of the above-mentioned Compound Example No. 7, and 10 g of a bisphenol Z-type polycarbonate resin (weight-average molecular weight = 50,000) were dissolved in 70 g of monochlorobenzene to prepare a coating liquid. The coating liquid was applied onto the above-mentioned charge generation layer by means of a wire bar and then dried at 110 °C for one hour to form a charge transport layer having a thickness of 19 microns, whereby an electrophotographic photosensitive member was prepared (Example 20).

The thus obtained photosensitive member was evaluated in the same manner as in Example 18.

The above-mentioned procedure was repeated except that Compound Example No. 28 was used for forming the charge transport layer thereby to prepare a photosensitive member (Example 21), which was then evaluated in the same manner as described above.

Further, the above-mentioned procedure was repeated except that the following Comparative Compound Examples 6 and 7 were respectively used for forming the charge transport layer (Comparative Examples 6 and 7), which were then evaluated in the same manner as described above.

### <Comparative Compound Examples>

The thus obtained results are shown in the following Table 6.

### Examples 22 and 23

3 g of 4-(4-dimethylaminophenyl)-2,6-diphenylthiapyrilium perchlorate, and 5 g of Compound Example No. 18 as a charge-transporting substance, and 5 g of a polyester resin (weight-average molecular weight = 49,000) were mixed with 50 g of a solvent comprising toluene and dioxane (1:1), and dispersed for 6 hours by means of a ball mill. The thus prepared dispersion was applied onto an aluminum sheet by means of a wire bar and then dried at 100 °C for 2 hours to form a photosensitive layer having a thickness of 15 microns, whereby an electrophotographic photosensitive member was prepared.

The thus obtained photosensitive member was evaluated in the same manner as in Example 1 (Example 22).

Separately, the above-mentioned procedure was repeated except that Compound Example No. 43 was used as the charge-transporting substance contained in the charge transport layer, thereby to prepare another electrophotographic photosensitive member. The thus prepared photosensitive member was evaluated in the same manner as described above (Example 23).

The thus obtained results are shown in the following Table 7.

### Examples 24 and 25

An aqueous ammonia solution of casein (comprising 11.2 g of casein, 1 g of 28 % ammonia water, and 222 ml of water) was applied onto an aluminum plate by means of a wire bar to form a primer layer having a thickness of 1 micron (after drying). On the primer layer, a charge transport layer and a charge generation layer were successively formed in the same manner as in Example 4, whereby an electrophotographic photosensitive member was prepared in the same manner as in Example 1 except that the laminate structure was different (Example 24).

The charging characteristics of the thus obtained photosensitive member were evaluated in the same manner as in Example 1 except that the charging polarity was positive.

The above procedure was repeated except that the charge transport layer was formed in the same manner as in Example 13 (Example 25).

The thus obtained results are shown in the following Table 8.

### Examples 26 and 27

A 5 % methanol solution of a soluble nylon (6-66-610-12 quaternary copolymer nylon) was applied onto an aluminum substrate to form a primer layer having a thickness of 0.5 micron (after drying).

Then, 5 of a pigment represented by the following formula:
was dispersed in 95 ml of tetrahydrofuran for 20 hours by means of a sand mill to prepare a dispersion.

Separately, 5 g of the above-mentioned Compound Example No. 14 as a charge-transporting substance, and 10 g of a bisphenol Z-type polycarbonate resin (weight-average molecular weight = 50,000) were dissolved in 30 ml of monochlorobenzene to prepare a solution. The solution was then added to the above-mentioned dispersion, and further dispersed by means of a sand mill for 2 hours, thereby to prepare a coating liquid. The thus prepared coating liquid was applied onto the above-mentioned primer layer by means of a wire bar and dried to form a photosensitive layer having a thickness of 20 microns (after drying), whereby an electrophotographic photosensitive member was prepared.

The electrophotographic characteristics of the thus obtained photosensitive member were evaluated in the same manner as in Example 1 (Example 26).

The above procedure was repeated except that Compound Example No. 32 was used as the charge-transporting substance (Example 27).

The thus obtained results are shown in the following Table 9.

## Claims (Claims for the following Contracting State(s): DE)

1. A photosensitive member for electrophotography, comprising an electroconductive substrate and a photosensitive layer disposed thereon, wherein the photosensitive layer comprises a triarylamine compound represented by the following general formula (I) or (II): wherein Ar₁ and Ar₂ respectively denote a biphenyl group capable of having a substituent; Ar₃ denotes an aromatic heterocyclic group capable of having a substituent; Ar₄ and Ar₅ respectively denote a benzene ring capable of having a substituent or aromatic fused-ring hydrocarbon group capable of having a substituent; R₁ and R₂ respectively denote a hydrogen atom, alkyl, alkoxyl or halogen atom; and at least one of Ar₄ and Ar₅ is an aromatic fused-ring hydrocarbon group.

2. A member according to Claim 1, wherein the photosensitive layer has a laminate structure comprising a charge generation layer and a charge transport layer.

3. A member according to Claim 2, which comprises the electroconductive substrate, and the charge generation layer and the charge transport layer in this order on the substrate.

4. A member according to Claim 2, which comprises the electroconductive substrate, and the charge transport layer and the charge generation layer in this order on the substrate.

5. A member according to Claim 2, wherein the charge transport layer comprises the compound represented by the formula (I) or (II), and an insulating polymer or organic photoconductive polymer.

6. A member according to Claim 2, wherein the charge transport layer comprises the compound represented by the formula (I) or (II), an insulating polymer or organic photoconductive polymer, and at least one species selected from the group consisting of a plasticizer, a surface lubricating agent, a potential stabilizing agent, and an anti-oxidizing agent.

7. A member according to Claim 2, wherein the charge generation layer comprises an organic charge-generating substance and an insulating resin.

8. A member according to Claim 1, which further comprises a primer layer disposed between the electroconductive substrate and the photosensitive layer.

9. A member according to Claim 1, which further comprises a protective layer disposed on the photosensitive layer.

10. A member according to claims 1 to 9, wherein the triarylamine compound is represented by the formula (I).

11. A member according to claims 1 to 9, wherein the triarylamine compound is represented by the formula (II).

## Claims (Claims for the following Contracting State(s): BE, CH, LI, ES, FR, GB, IT, NL, SE)

1. A photosensitive member for electrophotography, comprising an electroconductive substrate and a photosensitive layer disposed thereon, wherein the photosensitive layer comprises a triarylamine compound represented by the following general formula (I) or (II): wherein Ar₁ and Ar₂ respectively denote a biphenyl group capable of having a substituent; Ar₃ denotes a phenyl group capable of having a substituent or an aromatic heterocyclic group capable of having a substituent; Ar₄ and Ar₅ respectively denote a benzene ring capable of having a substituent or aromatic fused-ring hydrocarbon group capable of having a substituent; R₁ and R₂ respectively denote a hydrogen atom, alkyl, alkoxyl or halogen atom; and at least one of Ar₄ and Ar₅ is an aromatic fused-ring hydrocarbon group.

2. A member according to Claim 1, wherein the photosensitive layer has a laminate structure comprising a charge generation layer and a charge transport layer.

3. A member according to Claim 2, which comprises the electroconductive substrate, and the charge generation layer and the charge transport layer in this order on the substrate.

4. A member according to Claim 2, which comprises the electroconductive substrate, and the charge transport layer and the charge generation layer in this order on the substrate.

5. A member according to Claim 2, wherein the charge transport layer comprises the compound represented by the formula (I) or (II), and an insulating polymer or organic photoconductive polymer.

6. A member according to Claim 2, wherein the charge transport layer comprises the compound represented by the formula (I) or (II), an insulating polymer or organic photoconductive polymer, and at least one species selected from the group consisting of a plasticizer, a surface lubricating agent, a potential stabilizing agent, and an anti-oxidizing agent.

7. A member according to Claim 2, wherein the charge generation layer comprises an organic charge-generating substance and an insulating resin.

8. A member according to Claim 1, which further comprises a primer layer disposed between the electroconductive substrate and the photosensitive layer.

9. A member according to Claim 1, which further comprises a protective layer disposed on the photosensitive layer.

10. A member according to claims 1 to 9, wherein the triarylamine compound is represented by the formula (I).

11. A member according to claims 1 to 9, wherein the triarylamine compound is represented by the formula (II).

## Patentansprüche (Patentansprüche für folgende(n) Vertragsstaat(en): DE)

1. Lichtempfindliches Element für die Elektrofotografie, umfassend einen elektrisch leitenden Träger und eine lichtempfindliche Schicht, die darauf aufgebracht ist, worin die lichtempfindliche Schicht eine Triarylaminverbindung umfaßt, die durch die folgenden allgemeinen Formeln (I) oder (II) dargestellt ist: worin Ar₁ und Ar₂ jeweils eine Biphenylgruppe bedeuten, die in der Lage ist, einen Substituenten zu tragen, Ar₃ eine aromatische heterocyclische Gruppe, die in der Lage ist, einen Substituenten zu tragen, bedeutet, Ar₄ und Ar₅ jeweils einen Benzolring, der in der Lage ist, einen Substituenten zu tragen, oder eine aromatische Kohlenwasserstoffgruppe aus kondensierten Ringen, die in der Lage ist, einen Substituenten zu tragen, bedeuten, R₁ und R₂ jeweils ein Wasserstoffatom, eine Alkylgruppe, eine Alkoxygruppe oder ein Halogenatom bedeuten und wenigstens eine der beiden Gruppen Ar₄ und Ar₅ eine aromatische Kohlenwasserstoffgruppe aus kondensierten Ringen darstellt.

2. Element nach Anspruch 1, worin die lichtempfindliche Schicht eine Laminatstruktur aufweist, die eine Ladungserzeugungsschicht und eine Ladungstransportschicht umfaßt.

3. Element nach Anspruch 2, das einen elektrisch leitenden Träger und die Ladungserzeugungsschicht und die Ladungstransportschicht in dieser Reihenfolge auf dem Träger umfaßt.

4. Element nach Anspruch 2, das einen elektrisch leitenden Träger und die Ladungstransportschicht und die Ladungserzeugungsschicht in dieser Reihenfolge auf dem Träger umfaßt.

5. Element nach Anspruch 2, worin die Ladungstransportschicht die Verbindung, die durch die Formel (I) oder (II) dargestellt ist, und ein isolierendes Polymer oder ein organisches, lichtleitendes Polymer umfaßt.

6. Element nach Anspruch 2, worin die Ladungstransportschicht die Verbindung, die durch die Formel (I) oder (II) dargestellt ist, und ein isolierendes Polymer oder ein organisches, lichtleitendes Polymer und wenigstens eine Spezies, die aus der Gruppe, bestehend aus einem Plastifiziermittel, einem Oberflächengleit mittel, einem potentialstabilisierenden Mittel und einem Antioxidanzmittel, umfaßt.

7. Element nach Anspruch 2, worin die Ladungserzeugungsschicht eine organische, ladungserzeugende Verbindung und ein isolierendes Harz umfaßt.

8. Element nach Anspruch 1, das weiter eine Grundierschicht umfaßt, die zwischen dem elektrisch leitenden Träger und der lichtempfindlichen Schicht aufgebracht ist.

9. Element nach Anspruch 1, das weiter eine Schutzschicht umfaßt, die auf der lichtempfindlichen Schicht aufgebracht ist

10. Element nach einem der Ansprüche 1 bis 9, worin die Triarylaminverbindung durch die Formel (I) dargestellt ist.

11. Element nach einem der Ansprüche 1 bis 9, worin die Triarylaminverbindung durch die Formel (II) dargestellt ist.

## Patentansprüche (Patentansprüche für folgende(n) Vertragsstaat(en): BE, CH, LI, ES, FR, GB, IT, NL, SE)

1. Lichtempfindliches Element für die Elektrofotografie, umfassend einen elektrisch leitenden Träger und eine lichtempfindliche Schicht, die darauf aufgebracht ist, worin die lichtempfindliche Schicht eine Triarylaminverbindung umfaßt, die durch die folgenden allgemeinen Formeln (I) oder (II) dargestellt ist: worin Ar₁ und Ar₂ jeweils eine Biphenylgruppe bedeuten, die in der Lage ist, einen Substituenten zu tragen, Ar₃ eine Phenylgruppe, die in der Lage ist, einen Substituenten zu tragen, oder eine aromatische heterocyclische Gruppe, die in der Lage ist, einen Substituenten zu tragen, bedeutet, Ar₄ und Ar₅ jeweils einen Benzolring, der in der Lage ist, einen Substituenten zu tragen, oder eine aromatische Kohlenwasserstoffgruppe aus kondensierten Ringen, die in der Lage ist, einen Substituenten zu tragen, bedeuten, R₁ und R₂ jeweils ein Wasserstoffatom, eine Alkylgruppe, eine Alkoxygruppe oder ein Halogenatom bedeuten und wenigstens eine der beiden Gruppen Ar₄ und Ar₅ eine aromatische Kohlenwasserstoffgruppe aus kondensierten Ringen darstellt.

2. Element nach Anspruch 1, worin die lichtempfindliche Schicht eine Laminatstruktur aufweist, die eine Ladungserzeugungsschicht und eine Ladungstransportschicht umfaßt.

3. Element nach Anspruch 2, das einen elektrisch leitenden Träger und die Ladungserzeugungsschicht und die Ladungstransportschicht in dieser Reihenfolge auf dem Träger umfaßt.

4. Element nach Anspruch 2, das einen elektrisch leitenden Träger und die Ladungstransportschicht und die Ladungserzeugungsschicht in dieser Reihenfolge auf dem Träger umfaßt.

5. Element nach Anspruch 2, worin die Ladungstransportschicht die Verbindung, die durch die Formel (I) oder (II) dargestellt ist, und ein isolierendes Polymer oder ein organisches, lichtleitendes Polymer umfaßt.

6. Element nach Anspruch 2, worin die Ladungstransportschicht die Verbindung, die durch die Formel (I) oder (II) dargestellt ist, und ein isolierendes Polymer oder ein organisches, lichtleitendes Polymer und wenigstens eine Spezies, die aus der Gruppe, bestehend aus einem Plastifiziermittel, einem Oberflächengleitmittel, einem potentialstabilisierenden Mittel und einem Antioxidanzmittel, umfaßt.

7. Element nach Anspruch 2, worin die Ladungserzeugungsschicht eine organische, ladungserzeugende Verbindung und ein isolierendes Harz umfaßt.

8. Element nach Anspruch 1, das weiter eine Grundierschicht umfaßt, die zwischen dem elektrisch leitenden Träger und der lichtempfindlichen Schicht aufgebracht ist.

9. Element nach Anspruch 1, das weiter eine Schutzschicht umfaßt, die auf der lichtempfindlichen Schicht aufgebracht ist.

10. Element nach einem der Ansprüche 1 bis 9, worin die Triarylaminverbindung durch die Formel (I) dargestellt ist.

11. Element nach einem der Ansprüche 1 bis 9, worin die Triarylaminverbindung durch die Formel (II) dargestellt ist.

## Revendications (Revendications pour l'(les) Etat(s) contractant(s) suivant(s): DE)

1. Elément photosensible pour l'électrophotographie, comprenant un substrat électroconducteur et une couche photosensible disposée sur ce substrat, la couche photosensible comprenant un composé du type d'une triarylamine représenté par la formule générale (I) ou (II) suivante : dans laquelle Ar₁ et Ar₂ désignent respectivement un groupe biphényle capable de porter un substituant ; Ar₃ désigne un groupe hétérocyclique aromatique capable de porter un substituant ; Ar₄ et Ar₅ désignent respectivement un noyau benzénique capable de porter un substituant, ou un noyau hydrocarboné aromatique à noyaux condensés capable de porter un substituant ; R₁ et R₂ désignent respectivement un atome d'hydrogène, un groupe alkyle, alkoxyle ou un atome d'halogène ; et l'un au moins de Ar₄ et Ar₅ est un groupe hydrocarboné aromatique à noyaux condensés.

2. Elément suivant la revendication 1, dans lequel la couche photosensible a une structure stratifiée comprenant une couche génératrice de charges et une couche de transport de charges.

3. Elément suivant la revendication 2, qui comprend le substrat électroconducteur sur lequel se trouvent, dans l'ordre, la couche génératrice de charges et la couche de transport de charges.

4. Elément suivant la revendication 2, qui comprend le substrat électroconducteur sur lequel se trouvent, dans l'ordre, la couche de transport de charges et la couche génératrice de charges.

5. Elément suivant la revendication 2, dans lequel la couche de transport de charges comprend le composé représenté par la formule (I) ou (II) et un polymère isolant ou un polymère organique photoconducteur.

6. Elément suivant la revendication 2, dans lequel la couche de transport de charges comprend le composé représenté par la formule (I) ou (II), un polymère isolant ou un polymère organique photoconducteur, et au moins une substance choisie dans le groupe comprenant un plastifiant, un agent lubrifiant de surface, un agent de stabilisation de potentiel et un agent antioxydant.

7. Elément suivant la revendication 2, dans lequel la couche génératrice de charges comprend une substance organique engendrant des charges et une résine isolante.

8. Elément suivant la revendication 1, qui comprend en outre une première couche disposée entre le substrat électroconducteur et la couche photosensible.

9. Elément suivant la revendication 1, qui comprend en outre une couche protectrice disposée sur la couche photosensible.

10. Elément suivant les revendications 1 à 9, dans lequel le composé du type d'une triarylamine est représenté par la formule (I).

11. Elément suivant les revendications 1 à 9, dans lequel le composé du type d'une triarylamine est représenté par la formule (II).

## Revendications (Revendications pour l'(les) Etat(s) contractant(s) suivant(s): BE, CH, LI, ES, FR, GB, IT, NL, SE)

1. Elément photosensible pour l'électrophotographie, comprenant un substrat électroconducteur et une couche photosensible disposée sur ce substrat, la couche photosensible comprenant un composé du type d'une triarylamine représenté par la formule générale (I) ou (II) suivante : dans laquelle Ar₁ et Ar₂ désignent respectivement un groupe biphényle capable de porter un substituant ; Ar₃ désigne un groupe phényle capable de porter un substituant ou un groupe hétérocyclique aromatique capable de porter un substituant ; Ar₄ et Ar₅ désignent respectivement un noyau benzénique capable de porter un substituant, ou un groupe hydrocarboné aromatique à noyaux condensés capable de porter un substituant ; R₁ et _{R2} désignent respectivement un atome d'hydrogène, un groupe alkyle, alkoxyle ou un atome d'halogène ; et l'un au moins de Ar₄ et Ar₅ est un groupe hydrocarboné aromatique à noyaux condensés.

2. Elément suivant la revendication 1, dans lequel la couche photosensible a une structure stratifiée comprenant une couche génératrice de charges et une couche de transport de charges.

3. Elément suivant la revendication 2, qui comprend le substrat électroconducteur sur lequel se trouvent, dans l'ordre, la couche génératrice de charges et la couche de transport de charges.

4. Elément suivant la revendication 2, qui comprend le substrat électroconducteur sur lequel se trouvent, dans l'ordre, la couche de transport de charges et la couche génératrice de charges.

5. Elément suivant la revendication 2, dans lequel la couche de transport de charges comprend le composé représenté par la formule (I) ou (II) et un polymère isolant ou un polymère organique photoconducteur.

6. Elément suivant la revendication 2, dans lequel la couche de transport de charges comprend le composé représenté par la formule (I) ou (II), un polymère isolant ou un polymère organique photoconducteur, et au moins une substance choisie dans le groupe comprenant un plastifiant, un agent lubrifiant de surface, un agent de stabilisation de potentiel et un agent antioxydant.

7. Elément suivant la revendication 2, dans lequel la couche génératrice de charges comprend une substance organique engendrant des charges et une résine isolante.

8. Elément suivant la revendication 1, qui comprend en outre une première couche disposée entre le substrat électroconducteur et la couche photosensible.

9. Elément suivant la revendication 1, qui comprend en outre une couche protectrice disposée sur la couche photosensible.

10. Elément suivant les revendications 1 à 9, dans lequel le composé du type d'une triarylamine est représenté par la formule (I).

11. Elément suivant les revendications 1 à 9, dans lequel le composé du type d'une triarylamine est représenté par la formule (II).
